

March 10, 1925.

1,529,354

A. M. HAMBLET

METHOD OF MAKING ARTICLES FROM FIBROUS COMPOSITION

Filed Sept. 16, 1922



INVENTOR  
ABEL M. HAMBLET  
BY  
*R. B. T. [Signature]*  
ATTORNEY

Patented Mar. 10, 1925.

1,529,354

# UNITED STATES PATENT OFFICE.

ABEL M. HAMBLET, OF AKRON, OHIO, ASSIGNOR TO THE GOODYEAR TIRE & RUBBER COMPANY, OF AKRON, OHIO, A CORPORATION OF OHIO.

## METHOD OF MAKING ARTICLES FROM FIBROUS COMPOSITION.

Application filed September 16, 1922. Serial No. 588,644.

*To all whom it may concern:*

Be it known that I, ABEL M. HAMBLET, a citizen of the United States, and resident of Akron, Ohio, have invented new and useful Improvements in Methods of Making Articles from Fibrous Composition, of which the following is a specification.

My invention pertains to a method of making articles from a fibrous composition, and it has particular relation to a method of molding such articles.

The object of my invention is to provide a novel method of the above designated character which shall be simple and inexpensive to practice, and which shall provide articles having good wearing surfaces which offer a relatively great resistance to tearing or to separation into laminations.

Heretofore, it has been customary, in the manufacture of certain articles, such, for example, as the soles of shoes, which is contemplated by my present invention, to make the same by means of Fourdrinier machines, commonly used in the manufacture of paper. Articles made from this material must necessarily be punched or cut from a sheet in which form it must be made continuously in order to be efficient, leaving a relatively large proportion of waste material when the contour of the object being made is irregular. In the manufacture of soles for shoes, it is desirable that the sole and heel be unitary and that the instep portion be materially thinner than is the sole. When punched or cut from sheet material, this advantage cannot be secured as the entire sheet must be of the same thickness.

In material manufactured by the ordinary Fourdrinier machine the fibers are disposed in a single plane parallel to the wearing surface. Material made by this method offers comparatively small resistance to being separated into layers or laminations.

By my invention I have provided a method which eliminates the necessity of the use of a Fourdrinier machine, which is comparatively inexpensive, and which produces an article in which the fibers are disposed in all directions, thus providing a good wearing surface and offering a very high resistance to tearing. Also, no material whatsoever is wasted and the several portions of the article being manufactured can be made of any desired thickness.

The accompanying drawing is a perspective view of a machine for making soles for shoes, illustrating one form which my invention may assume.

In the drawing I show a container 3 connected, by means of a conduit 4 to a mold 5, the walls of which are composed of non-porous material, preferably impervious to liquid. In the drawing the mold 5 is of the form of a sole of a shoe, and consists of two similar plate members 6 each having a contour similar to that of the shoe sole to be formed. The members 6 are connected together at their edges by means of a curved side wall member 7. The walls 6 are removable from the curved member 7 and are held in position with respect thereto by means of clamping devices 8.

While the side wall 7 is illustrated as being comparatively high, it will be understood that the material is originally made relatively thick and is compressed to the proper thickness by means of a suitable pressure applying apparatus, not shown. It will be noted that the side wall 7 is narrower in the instep portion of the sole than in either the heel or sole portion. The object of this construction is to make the instep of the sole thinner than the sole and heel portion, so that, when a uniform pressure is exerted upon the entire face of the member, the instep portion of the finished member will be of the desired thickness.

Within the container 3 is disposed a quantity of wet fibers. These fibers are admitted to the mold 5 through the conduit 4 by the suitable operation of a valve member 9. After the mold is packed full with the fibers either by means of the pressure head of the fibers in the container 3, or by tamping, the valve 9 is closed. The mold is then opened and the molded article removed. It is next subjected to a heat treatment so as to dry the wet fibers contained therein. The pressure with which the fibers were forced into the mold causes them to stick together in the form into which they were molded after being removed therefrom.

In practicing my invention, I prefer to employ rubber coated fibers. These fibers are prepared by precipitating rubber in solution upon fibers suspended and dispersed therein. I prefer to subject the rubber coated fibers to a washing or displac-

ing treatment consisting of a series of baths with precipitating liquids, the last bath preferably being with a liquid consisting of approximately 60% alcohol and 40% 5 toluol.

It is a fact that alcohol and toluol constitute an azeotropic mixture, evaporating in approximately equal proportions of alcohol and toluol, irrespective of the relative quantities of the two liquids in the mixture, within certain limits. The particles of rubber, and the fibers on which they are deposited, retain a certain amount of the liquid in which they were immersed, so that, 10 upon drying the fibers, it is highly desirable that the alcohol content exceed the toluol content so that the liquid remaining in the fibers and the rubber, at any stage of the evaporation process, will comprise an excess 15 of alcohol, which is a precipitant of rubber. This is highly desirable owing to the fact that if the liquid remaining at any stage in the course of drying the fibers should be a solvent of rubber, the coating 20 on the fibers would be dissolved, the rubber in center of the mass would migrate to the surface, and the bond between the fibers would be destroyed.

The fibers, after being coated with rubber in the original precipitating mixture, are strained therefrom, either in a drum washer, or, if desired, in a Fourdrinier machine, and treated with the displacing liquids, before being placed in the container 3. I have 30 found that the most feasible proportions to employ, so as to produce a high grade mat with a minimum of manufacturing expense consists of a mass of which approximately 10% of the weight thereof is composed by 35 the fibers, and the rubber, and the remaining 90% by the 60% alcohol 40% toluol mixture with which they are impregnated. If the Fourdrinier machine is employed for straining and washing the fibers, they should 40 be thoroughly stirred and mixed before being placed in the mold 3, in order to cause 45 the fibers to extend in all directions.

It will be obvious that with the mixed up fibers forced into the mold 6, the fibers will 50 assume all manner of different positions, thus providing an article which will offer a high resistance to any tearing action or any tendency to separate the material into laminations. It will also be apparent that 55 on account of the fact that the fibers are forced directly into a suitable mold rather than being cut from a sheet, that absolutely no waste of fibers will occur during the various manufacturing steps.

60 Although I have shown but a single form of my invention and have described in detail but a single application thereof, it will be apparent to those skilled in the art that it is not so limited, but that various minor 65 modifications and changes may be made

therein without departing from the spirit of my invention or from the scope of the appended claims.

What I claim is:

1. The method of making articles from fibrous material which comprises precipitating a coating of rubber on a quantity of fibers, straining said fibers from the liquid, depositing a sufficient quantity of the wet fibers in a mold to fill the same, and drying 70 the fibers.

2. The method of making articles from fibrous material which comprises precipitating a coating of rubber on a quantity of fibers, straining said fibers from the liquid, 80 depositing a sufficient quantity of the wet fibers in a mold to fill the same, drying the fibers, and curing the rubber.

3. The method of making articles from fibrous material which comprises precipitating a coating of rubber on a quantity of fibers, straining said fibers from the liquid, depositing the wet fibers in a non-porous mold, removing the molded article from the mold and drying the same, and curing the 90 rubber.

4. The method of making an article from a fibrous material which comprises depositing a coating of rubber on a quantity of fibers and subsequently treating them with 95 a mixture of solvent and precipitant of such proportions that an excess of precipitant will remain after the evaporation of the solvent, and molding the fibers into the desired form.

5. The method of making an article from a fibrous material which comprises depositing a coating of rubber on a quantity of fibers and subsequently treating them with a mixture in which the proportion of precipitant to solvent is at least equal to azeotropic mixture requirements during the period of evaporation, and molding the fibers 100 to the desired form.

6. The method of making an article from a fibrous material which comprises depositing a coating of rubber on a quantity of fibers by means of a mixture of solvent and precipitant, and subsequently increasing the proportion of precipitant to solvent in the fibrous material so that the relative amount of precipitant to solvent is in excess of constant boiling point mixture requirements during the period of evaporation, and molding the fibers to the desired form.

7. The method of making a fibrous article 110 which comprises precipitating a coating of rubber on a quantity of fibers, subsequently treating them with a liquid comprising at least 50% alcohol, straining said fibers from the liquid, depositing the wet fibers in a mold having solid walls, and drying the product 115 in the mold.

8. The method of making a fibrous article 120 which comprises precipitating a coating of rubber on a quantity of fibers, treating them 125

with a liquid comprising at least 50% alcohol, straining said fibers from the liquid, depositing the wet fibers in a mold having solid walls, drying the product, and curing the rubber on the fibers.

9. The method of making a fibrous article which comprises precipitating a coating of rubber on a quantity of fibers, treating the fibers with a mixture consisting of more than 50% alcohol and less than 50% toluol, straining the rubber coated fibers from the liquid, and pressing them into a mold.

10. The method of making a fibrous article which comprises precipitating a coating of rubber on a quantity of fibers, treating the fibers with sufficient alcohol to form a liquid mixture in the fibrous material consisting of approximately 60% alcohol and

40% toluol, and molding them into the desired shape. 20

11. The method of making an article from a fibrous material which comprises precipitating a coating of rubber on a quantity of fibers from a mixture of rubber solvent and precipitant, and subsequently treating 25 said fibers with sufficient precipitant to ensure that a quantity thereof will remain in the fibers after the solvent is evaporated, and molding the fibers to the desired form.

In witness whereof, I have hereunto 30 signed my name in the presence of two subscribing witnesses.

ABEL M. HAMBLET.

Witnesses:

J. T. CHARLESON,  
F. A. LIND.